

# United States Patent [19]

Yamamoto et al.

[11] Patent Number: 4,741,863

[45] Date of Patent: May 3, 1988

[54] ALKALINE DEGREASING SOLUTION  
COMPRISING AMINE OXIDES

[75] Inventors: **Tsukasa Yamamoto; Asao Mochizuki**,  
both of Toyota; **Yoshikazu Shibata, Okazaki; Hiroshi Okita, Yokosuka; Koichi Ando, Sagamihara; Yasuhiro Okano, Ichikawa; Keiji Hadate, Chiryu**, all of Japan

[73] Assignees: **Toyota Jidosha Kabushiki Kaisha, Toyota; Nihon Parkerizing Company Limited**, Tokyo, both of Japan

[21] Appl. No.: 914,511

[22] Filed: Oct. 2, 1986

## Related U.S. Application Data

[63] Continuation of Ser. No. 699,164, Feb. 7, 1985, abandoned.

## Foreign Application Priority Data

Feb. 10, 1984 [JP] Japan 59-24104

[51] Int. Cl.<sup>4</sup> C11D 1/75; C11D 3/10

[52] U.S. Cl. 252/547; 134/40;  
252/528; 252/DIG. 14; 252/156

[58] Field of Search 134/40; 252/156, 528

## References Cited

### U.S. PATENT DOCUMENTS

3,223,647 12/1965 Drew et al. 252/547 X  
3,450,637 6/1969 Drew 252/528  
3,470,102 9/1968 Heinz 252/528  
3,668,153 6/1972 Crotty 252/528  
3,740,351 6/1973 Kaplan et al. 252/547  
3,843,563 10/1974 Davies et al. 252/547  
4,065,409 12/1977 Flanagan 252/528

4,174,304 11/1979 Flanagan 252/524  
4,276,205 6/1981 Ferry 252/528  
4,382,825 10/1983 McCready 134/2  
4,390,465 6/1983 Spekman 252/527  
4,457,322 7/1984 Rubin et al. 134/2

## FOREIGN PATENT DOCUMENTS

2758629 7/1978 Fed. Rep. of Germany .

Primary Examiner—Prince E. Willis  
Attorney, Agent, or Firm—Oblon, Fisher, Spivak,  
McClelland & Maier

## ABSTRACT

This invention relates to an aqueous solution of an alkaline degreasing agent employed for cleaning of metal products surface, and an alkaline degreasing agent employed for making up and replenishing the alkaline degreasing solution.

The essential constituent for these alkaline degreasing solution and agent is a compound, such as an alkyl dimethylamine oxide, a nonionic surface active agent, whose structural formula can be described as follows;



wherein R is an aliphatic hydrocarbon group having the number of carbon atoms 12-22.

The present alkaline degreasing solution can improve degreasing effects without lowering its deforming performance even at a low temperature.

17 Claims, 1 Drawing Sheet

FIG. 1



FIG. 2



**ALKALINE DEGREASING SOLUTION  
COMPRISING AMINE OXIDES**

This application is a continuation of application Ser. No. 699,164, filed Feb. 7, 1985 now abandoned.

**BACKGROUND OF THE INVENTION**

1. Field of the Invention

This invention generally relates to an aqueous solution of an alkaline degreasing agent, (hereinafter referred to as "an alkaline degreasing solution"), employed for removing oil and soil from surfaces of a steel sheet, galvanized steel sheet or galvannealed steel sheet, and an alkaline degreasing agent employed for making up and replenishing the alkaline degreasing solution. It relates more particularly to an alkaline degreasing solution with a low foaming tendency which are effective in a metal surface cleaning especially through a spray degreasing or immersion degreasing at a relatively low temperature such as 40° C., provided prior to a chemical conversion treatment and paint coating therefor.

2. Description of the Prior Art

Conventionally, metal products made of the aforementioned metals are generally treated by the following steps prior to paint coating:



The alkaline degreasing solutions and alkaline degreasing agents employed for cleaning metal surfaces have been introduced in various literature.

The alkaline degreasing agents are generally a powdery mixture of alkaline builders (alkaline compounds which are a main component of an alkaline degreasing agent), surface active agents, and defoaming agents.

The alkaline degreasing solution in which the alkaline degreasing agent is dissolved is employed for removing oil and soil from metal surfaces by means of a spray cleaning or immersion cleaning, the temperature of the solution employed for the cleaning generally being 40°-70° C. and degreasing time 1-10 minutes.

Recently, an interest has been increasingly generated in the alkaline degreasing agents and alkaline degreasing solutions utilized at a low temperature, with a view to energy conservation. The alkaline degreasing agents made for this purpose, however, have had the following deficiencies when they have been used for cleaning surfaces of metals (to be treated):

- a. excessive foaming during degreasing.
- b. low foaming but poor degreasing effects.

In the case that an alkaline degreasing solution excessively foams;

1. The foam may spill out of a degreasing tank and cause a loss of the alkaline degreasing solution in a large quantity, and

2. The foam may enter the inside of a box section of the metal products or of a box shaped metal product at the outset of an immersion degreasing. The foam left inside, due to the above shapes of the metal products, hinders the alkaline degreasing solution from contacting with inner surfaces thereof, and the foam whereby causes an incomplete degreasing on the inner surfaces.

**SUMMARY OF THE INVENTION**

A principal object of the invention is to provide an alkaline degreasing solution and alkaline degreasing agent, which improve degreasing effects without suppressing defoaming power so as to solve particularly the aforementioned problem b regarding the alkaline degreasing solution and alkaline degreasing agent used at a low temperature.

Another object of the present invention is to provide an alkaline degreasing solution and an alkaline degreasing agent with a low foaming tendency which are effective in a metal surface cleaning provided prior to a chemical conversion treatment and paint coating therefore, specially through a spray degreasing or immersion degreasing.

30 **BRIEF DESCRIPTION OF THE DRAWINGS**

FIG. 1 is a front view of the homomixer (T. K. Homomixer, TYPE: HU-M).

FIG. 2 is a front view of the apparatus for foaming test.

**DETAILED DESCRIPTION OF THE INVENTIONS**

40 The essential constituent for the alkaline degreasing solution and alkaline degreasing agent of the present invention is a compound, a nonionic surface active agent, whose structural formula can be described as follows;



45 R shown in the above structural formula represents aliphatic hydrocarbon group as hydrophobic group having the number of carbon atoms 12-22. The R may be an alkyl such as a dodecyl group ( $\text{C}_{12}\text{H}_{25}-$ ) or a octadecyl group ( $\text{C}_{18}\text{H}_{37}-$ ), or a combination thereof. Further the R may be of a synthetic, an extract or a derivative of natural materials, and either a linear or a branched hydrocarbon group. In addition, said R may be such an cis-9-Octadecenyl group that has an olefinic unsaturated combination, though the R is composed mainly of a saturated hydrocarbon group generally not containing an olefinic unsaturated group.

50 The R may be alkyl group obtained by hydrogenation of fatty acid, which can be a component of at least one of such natural vegetable oils as coconut oil, soybean oil, palm oil, sesami oil, sunflower oil, safflower oil and olive oil or such animal oils as lard and beef tallow. The R is mainly of saturated hydrocarbon group, however it may contain unsaturated hydrocarbon depending upon

the reduction conditions with hydrogen or others employed therefore.

The content of the compound in the alkaline degreas-  
ing solution or in alkaline degreasing agent of the inven-  
tion, shall be limited to 0.1-2 g/L (one liter of alkaline  
degreasing solution), and more preferably 0.1-1 g/L.  
The degreasing improvement effect of the degreas-  
ing performance of the compound, namely the dimethylam-  
ine oxide, is negligible in the case that the alkyl dimeth-  
ylamine content in the present alkaline degreas-  
ing solution is less than 0.1 g/L, particularly at a low tempera-  
ture, below 40 C. A satisfactory effect thereof can be  
obtained within the range of 0.1-1 g/L. Further the  
content of the compound in the present alkaline de-  
greasing solution is generally maintained within the  
range of 0.1-1 g/L, for the improvement effect thereof  
does not ameliorate in proportion to the amount thereof  
added up to 2 g/L. Therefore, the maximum content of  
the compound in the present alkaline degreas-  
ing solution should be 2 g/L.

The dimethylamine oxide itself (apart from other  
ingredients) may be added into a degreas-  
ing tank. However, in order to maintain 0.1-2 g of alkyl dimethylam-  
ine oxide content per one liter of the alkaline degreas-  
ing solution, preferably 0.1-1 g/L, it is prudent to mix the  
dimethylamine oxide with the other ingredients during  
the manufacturing stage thereof. The amount of alkyl  
dimethylamine oxide mixed in the alkaline degreas-  
ing agent should be 1-5% thereof.

Major ingredients, excluding the aforementioned  
dimethylamine oxide, contained in the alkaline degreas-  
ing solution and alkaline degreas-  
ing agent of the present  
invention are;

- (a) other surface active agents,
- (b) alkali builders, and

(c) defoaming agents, which are to be explained here-  
under. In addition, said (a) and (c) are not necessarily  
contained in the alkaline degreas-  
ing agent of the invention,  
and may be added thereto as other agents, when  
necessary.

#### (A) OTHER SURFACE ACTIVE AGENTS

Other surface active agents are not limited by a spe-  
cific ionic state, (i.e., nonionic, anionic, ampholytic, or  
cationic). Any surface active agent with the ionic state  
mentioned above may be employed therefor. However,  
the preferable surface active agent therefor should be a  
nonionic surface active agent (HLB 11-15, cloud point  
below 40° C., for example) or a mixture comprising a  
nonionic surface active agent and an anionic surface  
active agent.

As for the nonionic surface active agent, polyoxyeth-  
ylene alkylphenylether (alkylphenol type), polyoxyeth-  
ylene fatty acid ester (higher alcohol), etc., and prefera-  
bly polyoxyethylene nonylphenylether (HLB approxi-  
mately 12.6) may be employed.

As for the anionic surface active agent, -olefinic sul-  
fonate (-olefin type), alkyl sulfonate (normal paraffine  
type), alkyl sulfate, and alkylether sulfate (higher alcohol  
type), linear alkyl sulfonate (linear alkyl benzene type),  
and alkali salts of fatty acid, and preferably linear alkyl  
sulfonic acid and -olefinic sulfonate may be employed.

#### (B) ALKALINE BUILDER

The alkaline builder employed for the alkaline de-  
greasing solution and alkaline degreas-  
ing agent of the  
present invention shall not be specified in type. Alkaline  
builders may be generally classified into three types,

namely, the strong alkaline type composed mainly of  
sodium silicate or trisodium phosphate and/or caustic  
soda, medium alkaline type composed of one or more  
than one of the following; disodium phosphate, sodium  
pyrophosphate, sodium carbonate, etc., and mild alka-  
line type composed of disodium phosphate, sodium  
bicarbonate, sodium tripolyphosphate, sodium sesqui-  
carbonate, etc.. Any alkaline builder of the above types  
may be employed therefor.

#### (C) DEFOAMING AGENT

The defoaming agent employed for the alkaline de-  
greasing solution and alkaline degreas-  
ing agent of the  
present invention shall not be specified in type.

The present alkaline degreas-  
ing solution can improve  
degreasing effects without lowering its defoaming per-  
formance even at a low temperature, such as 40° C., due  
to the dimethylamine oxide contained therein as a com-  
ponent of the surface active agents therefor at a concen-  
tration 0.1-2 g/L.

The present alkaline degreas-  
ing solution can clean  
metal surfaces to be treated to a satisfactory degree,  
maintaining its defoaming performance, in approxi-  
mately one minute in such case that a spray method is  
employed therefor and in approximately two minutes  
by means of an immersion method, at a low tempera-  
ture, about 40° C.

Furthermore, the present alkaline degreas-  
ing solution can improve degreas-  
ing effects at a high temperature,  
above about 40° C., maintaining better defoaming per-  
formance in comparison with conventional alkaline  
degreasing solutions.

The present alkaline degreas-  
ing solution will show  
the above advantages more securely in the case that the  
hydrocarbon group of the dimethylamine oxide mixed  
therein is hydrogen reduced hydrocarbon obtained  
from a fatty acid composing natural vegetable oil such  
as palm oil or an animal oil, for the hydrocarbon group  
shall be of a straight chain as well as mixture of various  
groups.

The alkaline degreas-  
ing solution and alkaline de-  
greasing agent of the present invention may be added in  
with such surface active agents as nonionic surface  
active agents or a mixture comprising nonionic and  
anionic surface active agents in addition to the afore-  
mentioned to obtain the above advantages more securely.

The alkaline degreas-  
ing agent of the invention may  
be added in with the dimethylamine oxide along with  
alkali builders, said other surface active agents, defoam-  
ing agents, etc. to eliminate the troublesome task of  
adding separate alkyl dimethylamine oxide to an alka-  
line degreas-  
ing solution.

#### EMBODIMENTS OF THE INVENTION AND COMPARATIVE EXAMPLES

The present invention shall be explained in detail,  
with the embodiments of the invention being compared  
with comparative examples as follows:

##### (1) Alkaline Degreas- ing Agent

The alkaline degreas-  
ing agents, embodiments 1-6 and  
comparative examples 1-4 shown in Table 1, had been  
prepared as prescribed by means of a kneader utilized  
for an adequate mixing thereof.

The commercial products prescribed for the mixing  
materials are as follows:

## EXAMPLE

| MATERIALS         | MAKER                              | CONTENTS                                        |
|-------------------|------------------------------------|-------------------------------------------------|
| PERCOLENE Z       | Nihon Parkerizing Co., Ltd.        | surface conditioning agent including titanium.  |
| SOFT DETERGENT 60 | Lion Fats and Fatty Oils Co., Ltd. | linear alkyl benzene sodium sulfonate (anionic) |
| SURFYNOL 104      | Nissin Chemical Industry Co., Ltd. | nonionic surfactant                             |
| AROMOX DMC-W      | Lion Fats and Fatty Oils Co., Ltd. | alkyl dimethylamine oxide                       |
| COLORIN DF        | Sanyo Kasei Industry Co., Ltd.     | defoaming agent                                 |
| SN DEFORMER 5013  | San Nopco Ltd.                     | defoaming agent                                 |

## (2) Alkaline Degreasing Solution

18 g of the aforementioned alkaline degreasing agents were respectively solved in water so as to make one liter of an alkaline degreasing solution.

The alkaline degreasing agent will not be solved completely due to PERCOLENE Z mixed therein, and the alkaline degreasing solution, therefore will show slightly cloudy.

## (3) Test Panel and Rust Preventing Oil Application

A steel sheet was selected for the test panel to be applied with a rust preventing oil. A galvanized steel sheet and a galvannealed steel sheet may be applied with a rust preventing oil. However, the rust preventing oil applied on a galvanized steel sheet and galvannealed steel sheet are relatively easy to be degreased. Thus, a steel sheet was selected for the test panel.

Test panel: JIS—G—3141, SPCC

Rust preventing oil: DAPHNE OIL COAT (Idemitsu Kosan Co., Ltd.)

Rust preventing oil application:

The above rust preventing oil was applied on the surfaces of the test panels at 1-2 g/m<sup>2</sup> by means of a roll coater after the test panels had been cleaned with trichloroethylene.

Test panel A:

The test panel which was left at a room temperature for seven days after the application of the rust preventing oil as set forth above.

Test panel B:

The test panel which was left inside a high-temperature high-humidity cabinet at a temperature 60° C. ± 1° C. and relative humidity 95 ± 2%.

## (4) Degreasing Power Test

A test was conducted to evaluate degreasing performance of the alkaline degreasing solutions. Each alkaline degreasing solution was heated to be maintained at a temperature of 40° C. ± 1° C. Three test panels were immersed in each alkaline degreasing solution for two minutes, being placed therein separately so that they do not touch with each other, then were taken out of the solution to be rinsed off with a water spray for 30 seconds, and then were placed vertically at a room temperature for 60 seconds. Thereupon, water-wetted areas on the test panels were measured to evaluate degreasing performance of the alkaline degreasing solutions.

- 100—100% water-wetted. (degreasing performance: excellent)  
 5 50—50% water-wetted. (degreasing performance: poor)  
 The alkaline degreasing solutions, mixed with the abovementioned rust preventing oil were employed for the degreasing test. 2-3 g of the rust preventing oil was added to one liter of each alkaline degreasing solution to be mixed therein by means of a homomixer (T. K. HOMOMIXER; TYPE HU-M) shown in FIG. 1 at 10,000 rpm for 20 minutes.

## (5) Foaming Test

A foaming test was conducted, employing the testing apparatus shown in FIG. 2 in order to simulate the pump mixing at an actual immersion degreasing line, as follows:

- 20 2,000 ml of an alkaline degreasing solution 9 was provided in a 3-liter tall-beaker 11 (inside diameter 130 mm, height 300 mm) and then was placed in a thermostatic bath 12 to be maintained at a temperature of 40° C. ± 1° C. A turbine shaft 2 of a homomixer 8 was placed vertically in the tall beaker 11 at the center portion of the side-wall thereof. The bottom end portion of a stator 5 (a cylindrical ring encircling a turbine 4) was set at 60 mm above the bottom of the tall beaker 11. A plate 6, movable vertically, was moved along a supporting bar 3 to set the top side thereof with the same kevek of surface of the alkaline degreasing solution surface. The alkaline degreasing solution, maintained at a temperature of 40° C. ± 1° C., was agitated by means of the turbine 4 of the homomixer 8 at 10,000 rpm for 20 minutes to be pushed upward through the stator 5 to collide against the plate 6 to foam.

The thickness of the foam accumulated on the surface of the alkaline degreasing solution was measured in mm unit to evaluate the foaming tendency thereof after 30 seconds the homomixer 8 had stopped its rotating motion. The homomixer 8 was promptly taken out of the tall-beaker 11 after the alkaline degreasing solution had been agitated.

Embodiments of the invention are shown in Tables 1 and 2. Table 1 shows various example formula for alkaline degreasing agents in accordance with the present invention. Table 2 shows test results of various alkaline degreasing solutions prepared from the alkaline degreasing agents.

- 50 The results of comparisons between the embodiments 1-6 and comparative examples 1-4 can be summarized as follows:

## a. Degreasing Test

The degreasing test proved a superiority of the embodiments over the comparative examples. Each alkaline degreasing solution of the embodiments and comparative examples were maintained at a temperature of 40° C. ± 1° C. and wherein test panels A and B were respectively immersed for 2 minutes. In the case that the rust preventing oil was not added to the alkaline degreasing solutions, the embodiments showed slightly better results in comparison with the comparative examples. Whereas, in the case that the rust preventing oil was added to the alkaline degreasing solutions at mixture rates of 2 g/L and 3 g/L, the embodiments clearly showed better test results over the comparative examples at both mixture rates. The addition of the rust preventing oil to the embodiments up to 3 g/L caused a

minor decrease if any in their degreasing performance, while the decrease in the degreasing performance of the comparative examples caused by the rust preventing oil added up to 3 g/L was apparently noticeable.

b. Foaming Test

A forming test to compare the embodiments with the comparative examples as to their foaming shows the superiority of the embodiments. The embodiments with the rust preventing oil added therein showed excellent ( ) results. Some of the embodiments without the rust preventing oil showed good ( ) results. The comparative examples, with the rust preventing oil added therein showed various results, excellent ( ) to poor (X). The comparative examples, without the rust preventing oil showed a high foaming tendency. Furthermore, the embodiments also showed better results in individual comparisons thereof with the comparative examples.

1. An aqueous solution of an alkaline degreasing agent comprising at least inorganic alkaline builders, surface active agents and a defoaming agent comprising kerosine, for cleaning metal surfaces,

in which said surface active agents consist of two nonionic and one anionic surface active agents, wherein one nonionic comprises an alkyl dimethyl-amine oxide having the structural formula



wherein R is a hydrocarbon group having the number of carbon atoms in a range from 12 to 22, and the other nonionic comprises a polyoxyalkylene alkyl-phenylether or a polyoxyalkylene fatty acid ester;

TABLE 1

| COMPONENT (wt %)                     | EMBODIMENTS |      |      |      |      |      | COMPARATIVE EXAMPLE |      |      |      |
|--------------------------------------|-------------|------|------|------|------|------|---------------------|------|------|------|
|                                      | 1           | 2    | 3    | 4    | 5    | 6    | 1                   | 2    | 3    | 4    |
| <u>ALKALINE BUILDER</u>              |             |      |      |      |      |      |                     |      |      |      |
| sodium carbonate                     | 22.5        | 21.9 | 20.9 | 21.2 | 21.2 | 21.2 | 21.2                | 21.9 | 22.5 | 22.5 |
| sodium bicarbonate                   | 19.0        | 18.5 | 17.7 | 17.9 | 17.9 | 17.9 | 17.9                | 18.5 | 19.0 | 19.0 |
| disodium phosphate                   | 25.6        | 25.0 | 23.9 | 24.3 | 24.3 | 24.3 | 24.3                | 25.0 | 25.6 | 25.6 |
| trisodium phosphate                  | 5.1         | 5.0  | 4.8  | 4.9  | 4.9  | 4.8  | 4.9                 | 5.0  | 5.1  | 5.1  |
| sodium pyrophosphate                 | 2.1         | 2.0  | 1.9  | 1.9  | 1.9  | 1.9  | 1.9                 | 2.0  | 2.1  | 2.1  |
| sodium nitrite                       | 10.3        | 10.0 | 9.6  | 9.7  | 9.7  | 9.7  | 9.7                 | 10.0 | 10.3 | 10.3 |
| PARCOLENE Z                          | 5.1         | 5.0  | 4.8  | 4.9  | 4.9  | 4.8  | 4.9                 | 5.0  | 5.1  | 5.1  |
| <u>SURFACE ACTIVE AGENT</u>          |             |      |      |      |      |      |                     |      |      |      |
| polyoxyethylene                      | 4.6         | 4.6  | 4.6  | 4.6  | 6.7  | 6.7  | 4.6                 | 8.7  | 4.6  | 5.6  |
| nonylphenylether(nonionic)           |             |      |      |      |      |      |                     |      |      |      |
| (ethylene oxide: 8.6 mol, HLB: 12.6) |             |      |      |      |      |      |                     |      |      |      |
| SOFT DETERGENT 60                    |             |      |      |      |      |      | 1.0                 | 2.0  |      | 2.5  |
| SURFYNOL 104                         |             |      |      |      |      |      | 1.8                 | 1.8  |      | 1.8  |
| AROMOX DMC-W                         | 1.0         | 2.5  | 5.0  | 2.0  | 1.0  | 2.0  |                     |      |      |      |
| <u>DEFOAMING AGENT</u>               |             |      |      |      |      |      |                     |      |      |      |
| COLORIN DF                           |             |      |      |      |      |      |                     |      |      | 2.8  |
| SN DEFOAMER 5013                     | 2.8         | 3.6  | 4.9  | 2.8  | 2.8  | 4.9  | 2.8                 | 3.6  |      | 2.8  |
| kerosine                             | 1.9         | 1.9  | 1.9  | 1.9  | 1.9  | 1.9  | 1.9                 | 1.9  | 1.9  | 1.9  |
| Total                                | 100         | 100  | 100  | 100  | 100  | 100  | 100                 | 100  | 100  | 100  |

TABLE 2

| EMBODIMENTS         | ADDITION OF RUST PREVENTIVE OIL |                  |                  |                  |                        |                  |                  |                  |                        |                  |                  |                  |
|---------------------|---------------------------------|------------------|------------------|------------------|------------------------|------------------|------------------|------------------|------------------------|------------------|------------------|------------------|
|                     | 0                               |                  |                  |                  | 2 g/L                  |                  |                  |                  | 3 g/L                  |                  |                  |                  |
|                     | DEGREASING PERFORMANCE          |                  | DEFOAMING        |                  | DEGREASING PERFORMANCE |                  | DEFOAMING        |                  | DEGREASING PERFORMANCE |                  | DEFOAMING        |                  |
|                     | TEST PANEL A (%)                | TEST PANEL B (%) | PERFORMANCE (mm) | TEST PANEL A (%) | TEST PANEL B (%)       | PERFORMANCE (mm) | TEST PANEL A (%) | TEST PANEL B (%) | PERFORMANCE (mm)       | TEST PANEL A (%) | TEST PANEL B (%) | PERFORMANCE (mm) |
| 1                   | 100                             | 100              | 100              | 100              | 95                     | 100              | 0( )             | 100              | 95                     | 100              | 95               | 90               |
| 2                   | 100                             | 95               | 100              | 100              | 95                     | 95               | 0( )             | 100              | 100                    | 95               | 95               | 90               |
| 3                   | 100                             | 100              | 100              | 95               | 100                    | 100              | 0-3( )           | 100              | 100                    | 100              | 100              | 100              |
| 4                   | 100                             | 100              | 100              | 100              | 95                     | 100              | 0-3( )           | 100              | 100                    | 100              | 95               | 95               |
| 5                   | 100                             | 100              | 100              | 100              | 100                    | 100              | 0-3( )           | 100              | 100                    | 100              | 100              | 100              |
| 6                   | 100                             | 100              | 100              | 95               | 100                    | 100              | 0-3( )           | 100              | 100                    | 100              | 100              | 95               |
| COMPARATIVE EXAMPLE | 1                               | 90               | 90               | 90               | 90                     | 85               | 90               | 20(X)            | 90                     | 85               | 85               | 70               |
|                     | 2                               | 90               | 90               | 90               | 90                     | 90               | 95               | 5( )             | 70                     | 80               | 80               | 60               |
|                     | 3                               | 95               | 100              | 100              | 95                     | 100              | 95               | 5( )             | 90                     | 95               | 90               | 90               |
|                     | 4                               | 100              | 95               | 100              | 95                     | 95               | 95               | 5( )             | 95                     | 90               | 90               | 90               |

: Excellent

: Good

Δ: Fair

X: Poor

What is claimed is:

the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said nonionic surface active agent other than said amine oxide is 4.6 to 6.7 weight percent,

4.7 to 6.8 weight percent of said defoaming agent, and the remainder being said inorganic alkaline builders; and

in said alkaline degreasing aqueous solution prepared by adding water to said composition, the content of said alkyl dimethylamine oxide being 0.1 to 2 gram per one liter of said aqueous solution.

2. An aqueous solution of an alkaline degreasing agent as claimed in claim 1,

wherein said hydrocarbon group is an alkyl group.

3. An aqueous solution of an alkaline degreasing agent as claimed in claim 1,

wherein said hydrocarbon group is one obtained by hydrogenation of fatty acid of a natural vegetable oil.

4. An aqueous solution of an alkaline degreasing agent as claimed in claim 3,

wherein said natural vegetable oil is one selected from the group consisted of coconut oil, soybean oil, palm oil, sesami oil, sunflower oil, safflower oil, olive oil and the mixture thereof.

5. An aqueous solution of an alkaline degreasing agent as claimed in claim 1,

wherein said hydrocarbon group is one obtained by hydrogenation of fatty acid of an animal oil.

6. An aqueous solution of an alkaline degreasing agent as claimed in claim 1,

wherein said hydrocarbon group is one obtained by polymerization of ethylene monomer or a by de-composition of paraffin.

7. An aqueous solution of an alkaline degreasing agent as claimed in claim 1,

wherein the content of said alkyl dimethylamine oxide is 0.1 to 1 g per one liter of said aqueous solution.

8. An alkaline degreasing agent for making and replenishing an alkaline degreasing solution for cleaning of metal surface; comprising at least inorganic alkaline builders, surface active agents and a defoaming agent

comprising kerosine,

in which said surface active agents consist of two nonionic and one anionic surface active agents, wherein one nonionic comprises an alkyl dimethylamine oxide having the structural formula



wherein R is a hydrocarbon group having the number of carbon atoms in a range from 12 to 22, and the other nonionic comprises a polyoxyalkylene alkyl-phenylether or a polyoxyalkylene fatty acid ester; the composition ratios of said inorganic alkaline builders, defoaming agent and nonionic surface active agents being as follows, where all of the

solid portions thereof are determined in weight percent:

5.6 to 11.7 weight percent of said nonionic surface active agents, in which said amine oxide is 1 to 5 weight percent and said nonionic surface active agent other than said amine oxide is 4.6 to 6.7 weight percent,

4.7 to 6.8 weight percent of said defoaming agent, and the remainder being said inorganic alkaline builders.

9. An alkaline degreasing agent as claimed in claim 8, wherein said hydrocarbon group is an alkyl group.

10. An alkaline degreasing agent as claimed in claim

8,

wherein said hydrocarbon group is one obtained by hydrogenation of fatty acid of a natural vegetable oil.

11. An alkaline degreasing agent as claimed in claim

8,

wherein said hydrocarbon group is one obtained by hydrogenation of fatty acid of an animal oil.

12. An aqueous solution of an alkaline degreasing agent comprising at least inorganic alkaline builders, surface active agents and a defoaming agent comprising kerosine, for cleaning metal surfaces,

in which said surface active agents consist of two nonionic surface active agents, wherein one non-ionic comprises an alkyl dimethylamine oxide having the structural formula



wherein R is a hydrocarbon group having the number of carbon atoms in a range from 12 to 22 and the other nonionic comprises a polyoxyalkylene alkyl-phenylether or a polyoxyalkylene fatty acid ester; the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said polyoxyalkylene alkyl-phenylether or polyoxyalkylene fatty acid ester is 4.6 to 6.7 weight percent,

4.7 to 6.8 weight percent of said defoaming agent, and the remainder being said inorganic alkaline builders;

and in said alkaline degreasing aqueous solution prepared by adding water to said composition, the content of said alkyl dimethylamine oxide being 0.1 to 2 grams per one liter of said aqueous solution.

13. An alkaline degreasing agent for making and replenishing an alkaline degreasing solution for cleaning of metal surface; comprising at least inorganic alkaline builders, surface active agents and a defoaming agent comprising kerosine,

in which said surface active agents consist of two nonionic surface active agents, wherein one non-ionic comprises an alkyl dimethylamine oxide having the structural formula



wherein R is a hydrocarbon group having the number of carbon atoms in a range from 12 to 22, and the other nonionic comprises a polyoxyalkylene alkyl-phenylether or a polyoxyalkylene fatty acid ester; the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said polyoxyalkylene alkyl-phenylether or polyoxyalkylene fatty acid ester is 4.6 to 6.7 weight percent,

4.7 to 6.8 weight percent of said defoaming agent, and the remainder being said inorganic alkaline builders.

14. An aqueous solution of an alkaline degreasing agent comprising at least inorganic alkaline builders, 25 surface active agents and a defoaming agent comprising kerosine, for cleaning metal surfaces,

in which said surface active agents consist of three nonionic and one anionic surface active agents, wherein one nonionic comprises an alkyl dimethyl- 30 amine oxide having the structural formula



wherein R is a hydrocarbon group having the number of carbon atoms in a range from 12 to 22 and the other nonionic comprises a polyoxyalkylene alkyl-phenylether or a polyoxyalkylene fatty acid ester and another nonionic is a butyne diol nonionic surface active agent having the structural formula



wherein R<sub>6</sub> is an alkyl group having 4 to 6 carbon atoms.

15. An alkaline degreasing agent for making and replenishing an alkaline degreasing solution for cleaning of metal surface; comprising at least inorganic alkaline builders, surface active agents and a defoaming agent comprising kerosine,

in which said surface active agents consist of three nonionic and one anionic surface active agents, wherein one nonionic comprises an alkyl dimethyl- 55 amine oxide having the structural formula



wherein R is a hydrocarbon group having the number of carbon atoms in a range from 12 to 22, and the other nonionic comprises a polyoxyalkylene alkyl-phenylether or a polyoxyalkylene fatty acid ester

5

and another nonionic is a butyne diol nonionic surface active agent having the structural formula



wherein R<sub>6</sub> is an alkyl group having 4 to 6 carbon atoms;

the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said nonionic surface active agent other than said amine oxide is 4.6 to 6.7 weight percent,

4.7 to 6.8 weight percent of said defoaming agent, and the remainder being said inorganic alkaline builders.

16. An aqueous solution of an alkaline degreasing agent comprising at least inorganic alkaline builders, surface active agents and a defoaming agent comprising kerosine, for cleaning metal surfaces,

in which said surface active agents consist of three nonionic surface active agents, wherein one nonionic comprises an alkyl dimethylamine oxide having the structural formula



wherein R is a hydrocarbon group having the number of carbon atoms in a range from 12 to 22 and the other nonionic comprises a polyoxyalkylene alkyl-phenylether or a polyoxyalkylene fatty acid ester and another nonionic is a butyne diol nonionic surface active agent having the structural formula



35

wherein R<sub>6</sub> is an alkyl group having 4 to 6 carbon atoms;

the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said polyoxyalkylene alkyl-phenylether or polyoxyalkylene fatty acid ester is 4.6 to 6.7 weight percent,

4.7 to 6.8 weight percent of said defoaming agent and the remainder being said inorganic alkaline builders; and

in said alkaline degreasing aqueous solution prepared by adding water to said composition, the content of said alkyl dimethylamine oxide being 0.1 to 2 gram per one liter of said aqueous solution.

45

17. An alkaline degreasing agent for making and replenishing an alkaline degreasing solution for cleaning of metal surface; comprising at least inorganic alkaline builders, surface active agents and a defoaming agent comprising kerosine,

in which said surface active agents consist of three nonionic surface active agents, wherein one non-

60

65

ionic comprises an alkyl dimethylamine oxide having the structural formula



wherein R is a hydrocarbon group having the number 10 of carbon atoms in a range from 12 to 22, and the other nonionic comprises a polyoxyalkylene alkyl-phenylether or a polyoxyalkylene fatty acid ester, and another nonionic is a butyne diol nonionic 15 surface active agent having the structural formula



wherein R<sub>6</sub> is an alkyl group having 4 to 6 carbon atoms;

5 the composition ratios of said inorganic alkaline builders, defoaming agent and nonionic surface active agents being as follows, where all of the solid portions thereof are determined in weight percent:

5.6 to 11.7 weight percent of said nonionic surface active agents, in which said amine oxide is 1 to 5 weight percent and said polyoxyalkylene alkyl-phenylether or polyoxyalkylene fatty acid ester is 4.6 to 6.7 weight percent,

4.7 to 6.8 weight percent of said defoaming agent, and the remainder being said inorganic alkaline builders.

\* \* \* \* \*

20

25

30

35

40

45

50

55

60

65